



US011919061B2

(12) **United States Patent**  
**Komarasamy et al.**

(10) **Patent No.:** US 11,919,061 B2  
(45) **Date of Patent:** Mar. 5, 2024

(54) **SHEAR-ASSISTED EXTRUSION ASSEMBLIES AND METHODS**

(71) Applicant: **Battelle Memorial Institute**, Richland, WA (US)

(72) Inventors: **Mageshwari Komarasamy**, Richland, WA (US); **Scott A. Whalen**, West Richland, WA (US); **Brian K. Milligan**, Richland, WA (US)

(73) Assignee: **Battelle Memorial Institute**, Richland, WA (US)

(\*) Notice: Subject to any disclaimer, the term of this patent is extended or adjusted under 35 U.S.C. 154(b) by 0 days.

(21) Appl. No.: 17/944,932

(22) Filed: Sep. 14, 2022

(65) **Prior Publication Data**

US 2023/0078467 A1 Mar. 16, 2023

**Related U.S. Application Data**

(60) Provisional application No. 63/244,632, filed on Sep. 15, 2021.

(51) **Int. Cl.**  
**B21C 23/04** (2006.01)

(52) **U.S. Cl.**  
CPC ..... **B21C 23/04** (2013.01)

(58) **Field of Classification Search**  
CPC ..... B21C 23/04; B21C 23/002  
See application file for complete search history.

(56) **References Cited**

U.S. PATENT DOCUMENTS

|             |        |             |
|-------------|--------|-------------|
| 3,432,369 A | 3/1969 | Naastepad   |
| 3,640,657 A | 2/1972 | Rowe et al. |
| 3,661,726 A | 5/1972 | Denes       |

|             |         |                 |
|-------------|---------|-----------------|
| 3,684,593 A | 8/1972  | Benz et al.     |
| 3,884,062 A | 5/1975  | Green           |
| 3,892,603 A | 7/1975  | Reid            |
| 3,933,536 A | 1/1976  | Doser et al.    |
| 3,977,918 A | 8/1976  | Paladino et al. |
| 3,989,548 A | 11/1976 | Morris          |

(Continued)

FOREIGN PATENT DOCUMENTS

|    |             |         |
|----|-------------|---------|
| CN | 106140847 A | 11/2016 |
| CN | 107282671 A | 10/2017 |

(Continued)

OTHER PUBLICATIONS

WO PCT/US22/43532 Search Rept, dated Jan. 12, 2023, Battelle Memorial Institute.

(Continued)

*Primary Examiner* — Teresa M Ekiert

(74) *Attorney, Agent, or Firm* — Schwegman, Lundberg & Woessner, P.A.

(57) **ABSTRACT**

Shear-assisted extrusion assemblies are provided. The assemblies can include a billet containing assembly containing a billet comprising a billet outer material and a billet inner material in at least one cross-section; a tool operably engaged with the billet; an extrudate receiving channel configured to receive extrudate from the tool, wherein the extrudate comprises extruded outer material and extruded inner material in at least one cross-section, the extruded outer material being the same material as the billet outer material, and the extruded inner material being the same as the billet inner material. Methods for producing multi-material shear-assisted extrudate are also provided.

20 Claims, 23 Drawing Sheets



| (56)                  | References Cited |                   |                                                                                                                                                                                     |             |                     |
|-----------------------|------------------|-------------------|-------------------------------------------------------------------------------------------------------------------------------------------------------------------------------------|-------------|---------------------|
| U.S. PATENT DOCUMENTS |                  |                   |                                                                                                                                                                                     |             |                     |
| 4,287,749 A           | 9/1981           | Bachrach et al.   | 2016/0008918 A1                                                                                                                                                                     | 1/2016      | Burford             |
| 4,300,378 A           | 11/1981          | Thiruvarudchelvan | 2016/0151817 A1                                                                                                                                                                     | 6/2016      | Nayfeh et al.       |
| 4,585,473 A           | 4/1986           | Narasimhan et al. | 2016/0151818 A1                                                                                                                                                                     | 6/2016      | Shao                |
| 4,778,542 A           | 10/1988          | Clemens           | 2016/0167353 A1                                                                                                                                                                     | 6/2016      | Fan et al.          |
| 4,801,340 A           | 1/1989           | Inoue et al.      | 2016/0175981 A1                                                                                                                                                                     | 6/2016      | Kandasamy           |
| 4,808,224 A           | 2/1989           | Anderson et al.   | 2016/0175982 A1                                                                                                                                                                     | 6/2016      | Kandasamy et al.    |
| 4,892,596 A           | 7/1990           | Chatterjee        | 2016/0184922 A1                                                                                                                                                                     | 6/2016      | Kikyo               |
| 4,985,085 A           | 1/1991           | Chatterjee        | 2016/0228932 A1                                                                                                                                                                     | 8/2016      | Hayashi et al.      |
| 5,026,438 A           | 6/1991           | Young et al.      | 2016/0354860 A1                                                                                                                                                                     | 12/2016     | Boettcher et al.    |
| 5,089,060 A           | 2/1992           | Bradley et al.    | 2017/0008121 A1                                                                                                                                                                     | 1/2017      | Li                  |
| 5,242,508 A           | 9/1993           | McCallum et al.   | 2017/0136686 A1                                                                                                                                                                     | 5/2017      | Ueno et al.         |
| 5,262,123 A           | 11/1993          | Thomas et al.     | 2017/0163135 A1                                                                                                                                                                     | 6/2017      | Emberton et al.     |
| 5,283,130 A           | 2/1994           | Bradley et al.    | 2017/0182587 A1                                                                                                                                                                     | 6/2017      | Tokoro et al.       |
| 5,437,545 A           | 8/1995           | Hirai             | 2017/0216961 A1                                                                                                                                                                     | 8/2017      | Utter et al.        |
| 5,461,898 A           | 10/1995          | Lessen            | 2017/0225265 A1                                                                                                                                                                     | 8/2017      | Ito et al.          |
| 5,470,401 A           | 11/1995          | McCallum et al.   | 2017/0304933 A1                                                                                                                                                                     | 10/2017     | Miles et al.        |
| 5,492,264 A           | 2/1996           | Wadleigh          | 2017/0355003 A1                                                                                                                                                                     | 12/2017     | TenHouten et al.    |
| 5,737,959 A           | 4/1998           | Korbel et al.     | 2018/0036840 A1                                                                                                                                                                     | 2/2018      | Hu et al.           |
| 5,739,498 A           | 4/1998           | Sunamoto et al.   | 2018/0043467 A1                                                                                                                                                                     | 2/2018      | Huysmans            |
| 5,964,117 A           | 10/1999          | Holroyd et al.    | 2018/0050419 A1                                                                                                                                                                     | 2/2018      | Das et al.          |
| 5,988,484 A           | 11/1999          | Osborn et al.     | 2018/0311713 A1                                                                                                                                                                     | 11/2018     | Joshi et al.        |
| 6,022,424 A           | 2/2000           | Sellers et al.    | 2018/0354231 A1                                                                                                                                                                     | 12/2018     | Iwase               |
| 6,036,467 A           | 3/2000           | Jameson           | 2018/0369889 A1                                                                                                                                                                     | 12/2018     | Zhang et al.        |
| 6,638,462 B2          | 10/2003          | Davidson et al.   | 2019/0267153 A1                                                                                                                                                                     | 8/2019      | Kappagantula et al. |
| 6,843,405 B2          | 1/2005           | Okamoto et al.    | 2019/0275608 A1                                                                                                                                                                     | 9/2019      | Das et al.          |
| 6,940,379 B2          | 9/2005           | Creighton         | 2021/0086291 A1                                                                                                                                                                     | 3/2021      | Okada et al.        |
| 7,096,705 B2          | 8/2006           | Segal             | 2021/0205918 A1                                                                                                                                                                     | 7/2021      | Fujii et al.        |
| 7,314,670 B2          | 1/2008           | Bartsch et al.    | 2021/0252632 A1                                                                                                                                                                     | 8/2021      | Eller et al.        |
| 7,322,508 B2          | 1/2008           | Chang             | FOREIGN PATENT DOCUMENTS                                                                                                                                                            |             |                     |
| 7,954,692 B2          | 6/2011           | Fukuda            | EP                                                                                                                                                                                  | 2990178     | 8/2014              |
| 8,016,179 B2          | 9/2011           | Burford           | GB                                                                                                                                                                                  | 1258141     | 12/1971             |
| 8,240,540 B2          | 8/2012           | Tanaka et al.     | JP                                                                                                                                                                                  | 2003-275876 | 9/2003              |
| 8,313,692 B2          | 11/2012          | Somekawa et al.   | JP                                                                                                                                                                                  | 2007-222925 | 9/2007              |
| 8,695,868 B2          | 4/2014           | Messer et al.     | WO                                                                                                                                                                                  | WO          | 10/2019             |
| 10,189,063 B2         | 1/2019           | Lavender et al.   | PCT/US2019/040730                                                                                                                                                                   |             |                     |
| 10,369,748 B2         | 8/2019           | Whalen et al.     | WO                                                                                                                                                                                  | 2023043839  | 3/2023              |
| 10,695,811 B2         | 6/2020           | Joshi et al.      |                                                                                                                                                                                     |             |                     |
| 11,045,851 B2         | 6/2021           | Joshi et al.      |                                                                                                                                                                                     |             |                     |
| 2002/0029601 A1       | 3/2002           | Kwok              | OTHER PUBLICATIONS                                                                                                                                                                  |             |                     |
| 2004/0057782 A1       | 3/2004           | Okamoto et al.    | WO PCT/US22/43532 Written Opin, dated Jan. 12, 2023, Battelle Memorial Institute.                                                                                                   |             |                     |
| 2004/0238501 A1       | 12/2004          | Kawazoe et al.    | WO PCT/US2019/040730 IPRP, Jan. 5, 2021, Battelle Memorial Institute.                                                                                                               |             |                     |
| 2004/0265503 A1       | 12/2004          | Clayton et al.    | WO PCT/US2020/053168 IPRP, Apr. 7, 2022, Battelle Memorial Institute.                                                                                                               |             |                     |
| 2006/0005898 A1       | 1/2006           | Lui et al.        | WO PCT/US2020/053168 Search Rpt, dated Feb. 8, 2021, Battelle Memorial Institute.                                                                                                   |             |                     |
| 2006/0027628 A1       | 2/2006           | Sutherlin et al.  | WO PCT/US2020/053168 Written Opin, dated Feb. 8, 2021, Battelle Memorial Institute.                                                                                                 |             |                     |
| 2008/0029581 A1       | 2/2008           | Kumagai et al.    | WO PCT/US2021/050022 IPRP, Dec. 1, 2022, Battelle Memorial Institute.                                                                                                               |             |                     |
| 2008/0048005 A1       | 2/2008           | Forrest et al.    | WO PCT/US2021/050022 Search Rpt, dated Feb. 3, 2022, Battelle Memorial Institute.                                                                                                   |             |                     |
| 2008/0202653 A1       | 8/2008           | Ignberg           | WO PCT/US2021/050022 Weit. Opin., dated Feb. 3, 2022, Battelle Memorial Institute.                                                                                                  |             |                     |
| 2008/0251571 A1       | 10/2008          | Burford           | Abu-Farha, "A Preliminary Study on the Feasibility of Friction Stir Back Extrusion", Scripta Materials, 66, 2012, United States, 615-618.                                           |             |                     |
| 2009/0072007 A1       | 3/2009           | Nagano            | Amancio-Filho et al., "Joining of Polymers and Polymer-Metal Hybrid Structures: Recent Developments and Trends", Polymer Engineering & Science, 2009, United States, pp. 1461-1476. |             |                     |
| 2009/0269605 A1       | 10/2009          | Warke et al.      | Bozzi et al., "Intermetallic Compounds in Al 6016/IF-Steel Friction Stir Spot Welds", Materials Science and Engineering, 2010, Netherlands, pp. 4505-4509.                          |             |                     |
| 2009/0291322 A1       | 11/2009          | Watanabe et al.   | Cole et al., "Lightweight materials for Automotive Applications", Materials Characterization, 35, 1995, United States, pp. 3-9.                                                     |             |                     |
| 2010/0059151 A1       | 3/2010           | Iwamura et al.    | Evans et al., "Friction Stir Extrusion: A new process for joining dissimilar materials", Manufacturing Letters, 5, 2015, United States, pp. 25-28.                                  |             |                     |
| 2010/0089976 A1       | 4/2010           | Szymanski et al.  | Gann, J.A., "Magnesium Industry's Lightest Structural Metal", SAE Transactions, vol. 25-26, 1930-1931, United States, pp. 620-634, 641.                                             |             |                     |
| 2010/0132430 A1       | 6/2010           | Tsai et al.       |                                                                                                                                                                                     |             |                     |
| 2011/0104515 A1       | 5/2011           | Kou et al.        |                                                                                                                                                                                     |             |                     |
| 2011/0132970 A1       | 6/2011           | Nakagawa et al.   |                                                                                                                                                                                     |             |                     |
| 2011/0309131 A1       | 12/2011          | Hovanski et al.   |                                                                                                                                                                                     |             |                     |
| 2012/0006086 A1       | 1/2012           | Manchiraju et al. |                                                                                                                                                                                     |             |                     |
| 2012/0052322 A1       | 3/2012           | Hatakeyama et al. |                                                                                                                                                                                     |             |                     |
| 2012/0168045 A1       | 7/2012           | Ihara et al.      |                                                                                                                                                                                     |             |                     |
| 2012/0223451 A1       | 9/2012           | Hulseman et al.   |                                                                                                                                                                                     |             |                     |
| 2012/0258332 A1       | 10/2012          | Hatakeyama et al. |                                                                                                                                                                                     |             |                     |
| 2013/0075452 A1       | 3/2013           | Burford           |                                                                                                                                                                                     |             |                     |
| 2014/0000332 A1       | 1/2014           | Wilson et al.     |                                                                                                                                                                                     |             |                     |
| 2014/0002220 A1       | 1/2014           | Johnson et al.    |                                                                                                                                                                                     |             |                     |
| 2014/0076957 A1       | 3/2014           | Sayama et al.     |                                                                                                                                                                                     |             |                     |
| 2014/0102159 A1       | 4/2014           | Denison           |                                                                                                                                                                                     |             |                     |
| 2014/0102161 A1       | 4/2014           | Stewart           |                                                                                                                                                                                     |             |                     |
| 2014/0248508 A1       | 9/2014           | Ohhama et al.     |                                                                                                                                                                                     |             |                     |
| 2014/0283574 A1       | 9/2014           | Lavender et al.   |                                                                                                                                                                                     |             |                     |
| 2014/0291886 A1       | 10/2014          | Mark et al.       |                                                                                                                                                                                     |             |                     |
| 2014/0328710 A1       | 11/2014          | Cui et al.        |                                                                                                                                                                                     |             |                     |
| 2015/0075242 A1       | 3/2015           | Eller et al.      |                                                                                                                                                                                     |             |                     |
| 2015/0115019 A1       | 4/2015           | Pascal et al.     |                                                                                                                                                                                     |             |                     |
| 2015/0360317 A1       | 12/2015          | Kalvala et al.    |                                                                                                                                                                                     |             |                     |

(56)

**References Cited****OTHER PUBLICATIONS**

- Hammond et al., "Equal-Channel Angular Extrusion of a Low-Density High-Entropy Alloy Produced by High-Energy Cryogenic Mechanical Alloying", JOM. Vol. 66, No. 10, United States, 2014, pp. 2021-2029.
- Kaiser et al., "Anisotropic Properties of Magnesium Sheet AZ31", Materials Science Forum, vols. 419-422, Switzerland, 2003, pp. 315-320.
- Kuo et al., "Fabrication of High Performance Magnesium/Carbon-Fiber/PEEK/Laminated Composites", Materials Transactions, vol. 44, No. 8 (2003), Japan, pp. 1613-1619.
- Leitao et al., "Aluminum-steel lap joining by multipass friction stir welding", Materials and Design, 106, 2016, United States, pp. 153-160.
- Liu et al., "A Review of Dissimilar Welding Techniques for Magnesium Alloys to Aluminum Alloys", Materials, 7, 2014, United States, pp. 3735-3757.
- Liu et al., "Microstructure and mechanical properties of equimolar FeCoCrNi high entropy alloy prepared via powder extrusion", Intermetallics 75 (2016) , United States, pp. 25-30.
- Luo, Alan, "Magnesium: Current and Potential Automotive Applications", JOM, 54(2), 2002, United States, pp. 42-48.
- Martinsen et al., "Joining of Dissimilar Materials", CIRP Annals—Manufacturing Technology, 2015, United States, 21 pages.
- Nakamura et al., "Tool Temperature and Process Modeling of Friction Stir Welding", (2018) Modern Mechanical Engineering, 8, 78-94.
- Office Action for U.S. Appl. No. 14/222,468, filed Mar. 21, 2014, First named inventor Curtis A. Lavender, Notification date Nov. 6, 2015, 10 pages.
- Office Action for U.S. Appl. No. 14/222,468, filed Mar. 21, 2014, First named inventor Curtis A. Lavender, Notification date Apr. 1, 2016, 10 pages.
- Office Action for U.S. Appl. No. 14/222,468, filed Mar. 21, 2014, First named inventor Curtis A. Lavender, Notification date May 20, 2016, 3 pages.
- Office Action for U.S. Appl. No. 14/222,468, filed Mar. 21, 2014, First named inventor Curtis A. Lavender, Notification date Jan. 26, 2017, 9 pages.
- Office Action for U.S. Appl. No. 14/268,220, filed May 2, 2014, First Named Inventor Jun Cui, Notification date Dec. 1, 2015, 7 pages.
- Pickens, "Aluminum Powder Metallurgy Technology for High-Strength Applications", Journal of Materials Science 16 (1981) 1437-1457, United Kingdom, 21 pages.
- Rodewald et al. "Top Nd—Fe—B Magnets with Greater Than 56 MGoe Energy Density and 9.8 kOe Coercivity", IEEE Transactions on Magnetics, vol. 38, No. 5, 2002, United States, pp. 2955-2957.
- Saha, "Aluminum Extrusion Technology, Chapter 1, Fundamentals of Extrusion", The Materials Information Society, ASM International, 2000, United States, pp. 1-29.
- ThomasNet.com, <https://www.thomasnet.com/articles/custom-manufacturing-fabricating/friction-stir-welding/> Feb. 10, 2011 (Year: 2011).
- Trang et al., "Designing a Magnesium Alloy with High Strength and High Formability", Nature Communications, 2018, United Kingdom, 6 pages.
- Whalen et al., "High Ductility Aluminum Alloy Made from Powder by Friction Extrusion", Materialia 6 (2019) 100260, Netherlands, 6 pages.
- Whalen et al., U.S. Appl. No. 15/694,565, filed Sep. 1, 2017, titled "System and Process for Joining Dissimilar Materials and Solid-State Interlocking Joint with Intermetallic Interface Formed Thereby", 69 pages.
- Zhang et al., "Numerical Studies on Effect of Axial Pressure in Friction Stir Welding", (2007) Science and Technology of Welding and Joining, vol. 12, No. 3, United Kingdom, pp. 226-248.
- WO PCT/US2023/015228 Search Rpt, dated Jun. 15, 2023, Battelle Memorial Institute.
- WO PCT/US2023/015228 Written Opin, dated Jun. 15, 2023, Battelle Memorial Institute.





FIG. 3



FIG. 4



FIG. 5





FIG. 8



FIG. 9



FIG. 10



FIG. 11



FIG. 12



FIG. 13



FIG. 14



FIG. 15



FIG. 16



FIG. 17A



FIG. 17B



FIG. 17C



FIG. 17D



FIG. 17E



FIG. 18B

FIG. 18A



FIG. 18C



FIG. 19A



FIG. 19B



FIG. 19C



FIG. 19D



FIG. 20A



FIG. 20B



FIG. 20C



FIG. 20D



FIG. 20E



FIG. 21B

FIG. 21A



FIG. 21C

1100 Al (Outer material) and 2024 Al (Inner material)



FIG. 22A



FIG. 22B



FIG. 22C



FIG. 22D



FIG. 23A

FIG. 23B



FIG. 24A



FIG. 24B



FIG. 25A



FIG. 25B

FIG. 25C



FIG. 26A



FIG. 26B



FIG. 27



FIG. 28

## 1

## SHEAR-ASSISTED EXTRUSION ASSEMBLIES AND METHODS

## CROSS REFERENCE TO RELATED APPLICATION

This application claims priority to and the benefit of U.S. Provisional Patent Application Ser. No. 63/244,632 filed Sep. 15, 2021, entitled "Co-Extrusion/Cladding of Dissimilar AL Alloys Via Shear Assisted Processing and Extrusion", the entirety of which is incorporated by reference herein.

## STATEMENT AS TO RIGHTS TO INVENTIONS MADE UNDER FEDERALLY-SPONSORED RESEARCH AND DEVELOPMENT

This invention was made with Government support under Contract DE-AC05-76RL01830 awarded by the U.S. Department of Energy. The Government has certain rights in the invention.

## TECHNICAL FIELD

The present disclosure relates to extrusion assemblies and methods. Particular embodiments include shear-assisted extrusion assemblies and methods that can be used to create multi-metallic materials.

## BACKGROUND

Co-extrusion via hydrostatic extrusion and indirect extrusion is either expensive or results in non-uniform material flow. Furthermore, elaborate billet fabrication steps, requirement of specific area ratio between core and the sleeve, difficulty in co-extruding 1100 and 7075Al, and billet pre-heating are typically employed to obtain desirable bonding at the interface. Thermal spray coatings are limited to thin coatings which might not be beneficial for long-term applications due to cracking and spallation, and explosive bonding has safety and material constraints.

A few research level solutions that can never be applied at a manufacturing scale are fabrication of bi-metallic laminates using equal channel angular pressing and/or high pressure torsion.

Therefore, for increased energy efficiency and reduced plant downtime due to repair, an alternate manufacturing approach is required to fabricate the multi-metallic tubes with relative ease and better interface properties.

## SUMMARY

Shear-assisted extrusion assemblies are provided. The assemblies can include: a billet assembly containing a billet comprising a billet outer material and a billet inner material in at least one cross-section; a tool operably engaged with the billet; an extrudate receiving channel configured to receive extrudate from the tool, wherein the extrudate comprises extruded outer material and extruded inner material in at least one cross-section, the extruded outer material being the same material as the billet outer material, and the extruded inner material being the same as the billet inner material.

Methods for producing a multi-material shear-assisted extrudate are also provided. The methods can include: providing a billet comprising billet inner material and billet outer material; providing shear-assisted force to a tool operably engaged with the billet to form an extrudate

## 2

comprising extruded inner material and extruded outer material wherein the extruded outer material is the same material as the billet outer material, and the extruded inner material being the same as the billet inner material.

5

## DRAWINGS

Embodiments of the disclosure are described below with reference to the following accompanying drawings.

10 FIG. 1 is an example depiction of a portion of a shear-assisted extrusion assembly according to an embodiment of the disclosure.

15 FIG. 2 is a cross-section of an extrudate or extruded material according to an embodiment of the disclosure.

19 FIG. 3 is an example configuration of a portion of a shear-assisted assembly according to an embodiment of the disclosure.

20 FIG. 4 depicts another configuration of a portion of a shear-assisted extrusion assembly according to an embodiment of the disclosure.

25 FIG. 5 is a depiction of a shear-assisted extrudate according to an embodiment of the disclosure.

29 FIG. 6 is an exploded view of a billet configuration for use with shear-assisted extrusion assemblies according to an embodiment of the disclosure.

33 FIG. 7 is an extrudate material according to an embodiment of the disclosure.

30 FIGS. 8-12 are example billet configurations and commensurate extrudate materials obtained utilizing the example billet configurations according to embodiments of the disclosure.

35 FIG. 13 is a depiction of data of extruded material according to an embodiment of the disclosure.

39 FIG. 14 is a depiction of the operating conditions of a shear-assisted extrusion assembly utilizing differing materials according to an embodiment of the disclosure.

40 FIG. 15 is another example of shear-assisted extrusion assembly parameters according to an embodiment of the disclosure.

44 FIG. 16 is an example of co-metallic extruded material properties according to an embodiment of the disclosure.

48 FIGS. 17A-17E are depictions of multi-metallic extruded material according to an embodiment of the disclosure.

52 FIGS. 18A-18C are depictions of interfacial portions of multi-metallic extruded materials according to an embodiment of the disclosure.

56 FIGS. 19A-19D are depictions of multi-metallic extruded materials according to an embodiment of the disclosure.

59 FIGS. 20A-20E are depictions of interfacial multi-metallic extruded materials according to an embodiment of the disclosure.

63 FIGS. 21A-21C are depictions of portions of multi-metallic extruded materials according to an embodiment of the disclosure.

67 FIGS. 22A-22D are depictions of multi-metallic extruded materials according to an embodiment of the disclosure.

71 FIGS. 23A-23B are depictions of a billet configuration according to an embodiment of the disclosure.

74 FIGS. 24A-24B are depictions of billet configurations according to an embodiment of the disclosure.

78 FIGS. 25A-25C are depictions of multi-metallic extruded materials according to an embodiment of the disclosure.

82 FIGS. 26A-26B are depictions of multi-metallic extruded materials according to an embodiment of the disclosure.

86 FIG. 27 is a depiction of a multi-metallic extrudate according to an embodiment of the disclosure.

FIG. 28 is a depiction of a multi-metallic extrudate according to an embodiment of the disclosure.

## DESCRIPTION

This disclosure is submitted in furtherance of the constitutional purposes of the U.S. Patent Laws “to promote the progress of science and useful arts” (Article 1, Section 8).

The present disclosure will be described with reference to FIGS. 1-28. The present disclosure provides assemblies and methods for creating a co-extruded multi-metallic extrudates that can be co-extruded in the form of tubes. The extrudates can include at least an extruded inner material within an extruded outer material. The inner material can be referred to as a core and the outer material can be referred to as a cladding or sleeve. In tube configurations, the inner material can be referred to as an inner layer and the outer material as an outer layer.

The materials (inner, outer, intermediate) that make up the extrudate can have distinct chemical and/or mechanical properties. For example, co-extrusion of 6061 (shell) and 7075 (core), 1100 (shell) and 7075 (core), and 1100 (shell) and 2024 (core) was performed to complete extrudates having commensurate outer and inner materials having sound bonding at the interface. Furthermore, thickness of the sleeve and core can be controlled via the area ratio of the constituent billet material. Multi-metallic tubes can be fabricated utilizing a tool that engages a mandrel.

The ShAPE process works in billet area ratio of  $\frac{1}{3}$  and  $\frac{2}{3}$ , and also  $\frac{1}{2}$  and  $\frac{1}{2}$  leading to the tube thickness of  $\frac{1}{3}$  and  $\frac{2}{3}$ , and  $\frac{1}{2}$  and  $\frac{1}{2}$ , respectively. Based on the current observations, a much thinner core/sleeve, preferably having  $\frac{1}{4}$  of the tube thickness is quite possible. Therefore, either a thicker or thinner coating can easily be fabricated. Temperature control of the process using the shear and friction parameters can provide for more flexible fabrication of multi-metallic components having significantly different flow stresses. Furthermore, multi-metallic extrudate tubes exhibiting variable thicknesses can be fabricated by controlling the billet stack with minimal effort in billet fabrication. This allows for joining the b metallic tubes to other structures so that easily weldable material of necessary thickness is the sleeve. Difficult to extrude material combination such as 1100 and 7075/2024 Al can easily be co-extruded.

Furthermore, these multi-metallic extrudates, having gone through high temperature severe plastic deformation, can be aged without solutionizing or annealing heat treatments, thereby thermal stresses and the subsequent dimensional instability can be avoided and/or grain growth minimized.

Referring to FIG. 1, a portion of an example shear-assisted extrusion apparatus 10 is shown that includes a billet holder assembly 12 that comprises and container base 12a and a container ring 12b. Within assembly 12 is billet 20. Billet 20 comprises at least two materials, but may contain additional materials in different alignments. In this configuration, billet material 20 comprises at least a billet inner material 22b and a billet outer material 24b. As an example, materials 22b and 24b will be different materials as noted herein. The materials may differ in chemical and/or mechanical properties. The materials may also have different dimensions. For example, the thickness ratio of the materials as shown appear to be the same. Other thickness ratios can be utilized with the outer material being less or greater thickness than the inner material.

Tool 14 can be retained within tool holder 21 and operably engaged with billet material 20 to create a high shear region 26 at die face 28. As shown, a rotational force and axial force

is applied to die face 28 of tool 14. The axial force may be applied from the tool upon the feed material; alternatively, the axial force may be applied from the feed material upon the tool. In accordance with example implementations, the shear assisted extrusion process will provide an extrudate 18. Mandrel 16 can be anchored in billet holder assembly 12 and extend through billet material 20 and die face 28 to extrude receiving channel 11.

This application is related to U.S. Continuation-In-Part 10 patent application Ser. No. 17/473,178 filed Sep. 13, 2021, entitled “Devices and Methods for Performing Shear-Assisted Extrusion and Extrusion Processes”, the entirety of 15 which is hereby incorporated by reference herein.

Referring to FIG. 2, extrudate 18 can comprise at least 20 extruded inner material 22e and extruded outer material 24e. These extruded materials (22e/24e) can be the same as billet materials (22b/24b) and have substantially the same ratio of thickness (e.g., area ratio of  $\frac{1}{3}$  and  $\frac{2}{3}$ , and also  $\frac{1}{2}$  and  $\frac{1}{2}$ , leading to the tube thickness of  $\frac{1}{3}$  and  $\frac{2}{3}$ , and  $\frac{1}{2}$  and  $\frac{1}{2}$ , respectively). The extruded materials can be bonded at interface 23 while the billet materials are not bonded.

Referring to FIGS. 3-12, various combinations of billet material configurations as well as extruded material configurations are shown. For example, FIGS. 3-7 demonstrate 25 inner billet material 22b and outer billet material 24b bounded by billet material 40b. When shear-assisted extruded, extruded inner material 22e and outer extruded outer material 24e are bounded by extruded material 40e. This extruded material can have bonding interfaces between the inner 22e and outer 24e materials as well as between the outer 24e and extruded material 40e and/or the inner 22e and extruded material 40e.

Referring to FIGS. 8-12 a summary of example billet and 30 extruded material configurations are shown. This summary is not provided to be exhaustive, just as an example. Accordingly, the billet material and the extrudate can include intermediate materials 90b/90e. These intermediate materials can include multiple materials themselves. Thus, the materials can include multiple layers in at least one cross-section. Additionally, with reference to FIGS. 10 and 11, inner and/or outer materials can extend to complete and be the same material as bounding materials. Accordingly, the inner or outer materials can be the same as bounding materials (e.g., 40). Also, with reference to FIG. 12, multiple 35 inner and multiple outer materials can be provide as shown. Accordingly, outer materials can include distinct materials 24 and 120. Additionally, inner materials can include distinct materials 22 and 122. As the depiction provides, the abutment of these materials need not align.

Accordingly, billet containing assembly 12 containing a 40 billet that includes a billet outer material 22b and a billet inner material 24b in at least one cross-section. The billet 20 can also include a billet intermediate material 90b between billet inner material 22b and billet outer material 24b in the 45 at least one cross-section. The assembly can include mandrel 16 extending from billet containing assembly 12 to tool 14. Mandrel 16 can extend through an opening in die face 28 of the tool 14. Billet material 20 can also include a billet boundary material 40b directly adjacent and/or lateral of either billet inner material 22b or outer material 24b. the billet boundary material is the same material as the billet outer material. Billet boundary material 40b can be a different material than either or both of the billet inner material 22b or outer material 24b. In at least one cross-section the 50 thickness of one or more of the inner 22e, outer 24e, and/or intermediate 90b billet materials is different. Each material thickness can be as low as a  $10^{\text{th}}$  of the thickness of the

material directly adjacent thereto. In billet container assembly **12**, the billet materials can be unbound.

The extrudate **18** can also include extruded intermediate material **90e** between extruded outer material **24e** and extruded inner material **22e** in the at least one cross-section.

In accordance with the above assemblies, the methods can include a billet intermediate material **90b** between the billet inner material **22b** and billet outer material **24b**. Billet intermediate material **90b** can be a single material or multiple different materials. Inner **22b** and outer **24b** billet material can be about the same thickness in at least one cross-section. Extruded inner **22e** and outer **24e** materials can be about the same thickness in at least one cross-section. Inner billet material **22b** can be  $\frac{1}{10}$  to  $\frac{1}{10}$  the thickness of outer **24b** billet material. Extruded inner material **22e** can be  $\frac{1}{10}$  to  $\frac{1}{10}$  of the thickness of extruded outer billet material **24e**. The extruded materials define bonded interfaces between different and previously unbound billet materials.

As an example method with reference to Table 1 below, multi-metallic extrudates were prepared. These parameters are not limiting and ranges of rotational speed as well as advance rate can be utilized.

TABLE 1

| Summary of example shear-assisted processing conditions employed to fabricate the multi-material extrudates. |                            |                           |                 |
|--------------------------------------------------------------------------------------------------------------|----------------------------|---------------------------|-----------------|
| Material combination                                                                                         | Die rotational speed (RPM) | Die advance rate (mm/min) | Tube length, mm |
| 1100 (24) and 7050 (22) Al                                                                                   | 40                         | 60                        | 1960            |
| 1100 (24) and 2024 (22) Al                                                                                   | 45                         |                           | 1830            |

The extruded tubes were sectioned for various microscopy and mechanical property characterizations in as-extruded condition. For optical and scanning electron microscopy (SEM) analysis, the tubes were sectioned along both longitudinal and transverse cross-sections. The cut samples were mounted in an epoxy, polished to a surface finish of 0.05  $\mu\text{m}$  using colloidal silica suspension, and etched using Keller's reagent. Both stereo and light microscopy (in bright field mode) analyses of the samples were carried to analyze the tube quality and interface characteristics. The samples were repolished to 0.05  $\mu\text{m}$  surface finish for SEM and energy-dispersive X-ray spectroscopy (EDS) analysis. SEM in back scattered electron (BSE) mode and EDS analyses of the cladded tubes and the interface between 1100/7075 Al, and 1100/2024 Al were completed using the FEI Quanta 3D field emission gun dual beam FIB/SEM. Vickers hardness measurements in as-extruded was carried out using Clark Microhardness tester CM-700AT and five indents per sample was done. Tensile testing of 127 mm (5") long tubes was carried out in accordance with ASTM-B557 standard. All the results and discussion are presented in the next section.

Referring to FIG. 3, and with reference to Table 2, tensile properties of multi-metallic extrudates having differing inner and outer thickness ratios are shown.

TABLE 2

| Material combinations                            | YS (MPa) | UTS (MPa) | EI % |
|--------------------------------------------------|----------|-----------|------|
| 6061/7075 Al ( $\frac{1}{2}$ and $\frac{1}{2}$ ) | 175      | 252       | 13   |

TABLE 2-continued

| Material combinations                            | YS (MPa) | UTS (MPa) | EI % |
|--------------------------------------------------|----------|-----------|------|
| 6061/7075 Al ( $\frac{1}{2}$ and $\frac{1}{2}$ ) | 168      | 224       | 8.5  |
| 1100/7075 Al                                     | 132      | 219       | 9    |
| 1100/2024 Al                                     | 116      | 198       | 11.5 |

10 The measured tool temperature ( $^{\circ}\text{C}$ .) and the spindle torque (Nm) as a function of plunge depth for both the extrusions is presented in FIGS. 13 and 14, respectively. What can be considered a long steady-state temperature region was followed by an initial transient temperature region.

15 Steady-state temperatures in 1100/7075 Al and 1100/2024 Al were about 380 and 390  $^{\circ}\text{C}$ ., respectively, mainly due to slightly lower rotational speed in the former extrusion. An initial transition in spindle torque was also noted (FIG. 15) 20 followed by an almost steady-state. However, beyond plunge depth of  $\sim$ 40 mm, oscillation in torque was observed. Exact origin of these oscillations is not known; however, a possible hypothesis could be based on the sticking characteristics of 1100 Al exhibits during thermomechanical processing. During ShAPE process, 1100 Al sticks to the extrusion die and at higher force the material slips, then the continuation of this process would result in torque oscillations, as noted in FIG. 15.

25 Referring next to FIG. 16, a comparison of coextruded multi-metallics is shown. Additional analysis of coextruded materials have been performed using Stereo and light microscopy of cladded 1100 on 7075 Al and 1100 on 2024 Al are presented in FIGS. 17A-17E and 20A-20E respectively. FIGS. 17A-17B and 20A-20B represent the macro-view of both longitudinal and transverse cross-sections for cladded 1100/7075 Al and 1100/2024 Al, respectively. The cladded outer layer (1100 Al) was continuously present along the tube (dark region) in all the conditions and cross-sections analyzed. The bright inner region in FIGS. 30 17A-17B and 20A-20B correspond to 7075 Al and 2024 Al, respectively. Thickness of tubes measured on the transverse cross-section for 1100/7075 and 1100/2024 are  $0.92\pm0.05$  mm and  $0.97\pm0.14$  mm, respectively. As noted, tube thickness in 1100/2024 Al was higher than 1 mm in certain 35 locations as compared with 1100/7075 Al. The thickness of the outer and inner layers for 1100/7075 Al are  $0.6\pm0.1$  and  $0.36\pm0.06$  mm, respectively, and thickness for the outer and inner layers for 1100/2024 Al are  $0.57\pm0.1$  and  $0.38\pm0.03$  mm, respectively. In both the tubes, the 1100 Al outer layer 40 exhibited larger thickness than the expected 0.5 mm based on the billet area. The light microscopy images are presented in FIGS. 17B-17E and 20B-20E. Both outer and inner layers of the tube for both cladded configurations did not have any 45 processing flaws. Furthermore, higher magnification analysis of the interface region shows that the interface in both the conditions is defect-free and wavy in nature. SEM-BSE and SEM-EDS analyses of 1100/7075 and 1100/2024 Al cladded tubes are presented in FIGS. 18A-18C and 21A-21C, respectively. Interface region between 1100/7075 and 1100/2024 50 Al cladded tubes is marked with a solid arrow. For the most part, interface region did not exhibit discontinuities except for a few micro-cracks as marked by the dotted arrow in FIG. 18A. Therefore, the interface region was metallurgically bonded in both the conditions as clearly observed in 55 FIGS. 18B and 21B. Furthermore, presence of second phases is noted in both 7075 and 2024 Al alloys. Results of SEM-EDS line scan analysis of 1100/7075 Al and 1100/

2024 Al are presented in FIGS. 18C and 21C, respectively. As expected, Zn and Cu content increased across the cladded interface from 1100 Al into the 7075 and 2024 Al, respectively. Additional data are provided in Tables 3-4 below regarding hardness and tensile strength of the multi-metallic materials.

TABLE 3

| Hardness summary in as-extruded condition for 1100 and 7075 Al and 1100 and 2024 Al cladded tubes |                         |                  |
|---------------------------------------------------------------------------------------------------|-------------------------|------------------|
|                                                                                                   | Material identification | Hardness (HV0.1) |
| 1100/7075 Al                                                                                      | 1100 Al                 | 20.2 $\pm$ 0.2   |
|                                                                                                   | 7075 Al                 | 83.3 $\pm$ 3.0   |
| 1100/2024 Al                                                                                      | 2024 Al                 | 68.0 $\pm$ 1.0   |
|                                                                                                   | 1100 Al                 | 21.0 $\pm$ 0.3   |

TABLE 4

| Tensile properties Summary of the cladded Al tubes. |               |             |                |
|-----------------------------------------------------|---------------|-------------|----------------|
|                                                     | YS (MPa)      | UTS (MPa)   | EI. %          |
| 1100/7075 Al                                        | 135 $\pm$ 3.5 | 213 $\pm$ 5 | 6.4 $\pm$ 1.4  |
| 1100/2024 Al                                        | 117 $\pm$ 5.4 | 199 $\pm$ 4 | 10.6 $\pm$ 1.1 |

Overall, the presence of metallurgically bonded interface obtains cladded tubes with good structural integrity.

Referring next to FIGS. 19A-19D and 22A-22D, inner and outer materials having similar cross-section area are provided and metallurgical bonding was determined to be present in both cases of 1100 outer and 7075 or 2024 inner.

In accordance with an example implementation, at least a pair of billet designs are shown in FIGS. 23A-23B and 24A-24B. FIGS. 23A-23B demonstrate a similar thickness while FIGS. 24A-24B demonstrate an inner 1/3 to outer 2/3 ratio. The materials used were inner 7075 and outer 6061. In FIGS. 25A-28 analysis results of both FIGS. 23A-B and 24A-B designs are shown.

Successful extrudate fabrication of distinctly different flow strength materials can provide heat exchangers with high temperature strength materials having a corrosion/oxidation resistance material as either an inner or outer material. At least one example of this application is co-extrusion of copper-nickel bi-metallic tubing which has been performed using these methods. Moreover, the apparatus and methods described herein enable continuous cladding from start to stop. For example, the outer material can be present over an entirety of an extrudate surface. Additionally, or alternatively, the apparatus and method provide the ability to vary or change outer material thickness. That is, a thicker and/or thinner outer material may be continuously fabricated along an outer surface of the extrudate.

In compliance with the statute, embodiments of the invention have been described in language more or less specific as to structural and methodical features. It is to be understood, however, that the entire invention is not limited to the specific features and/or embodiments shown and/or described, since the disclosed embodiments comprise forms of putting the invention into effect. The invention is, therefore, claimed in any of its forms or modifications within the proper scope of the appended claims appropriately interpreted in accordance with the doctrine of equivalents.

The invention claimed is:

1. A shear assisted extrusion assembly, the assembly comprising:
  - a billet containing assembly configured for receiving a billet comprising a billet outer material and a billet inner material in at least one cross-section, wherein the billet outer material and the billet inner material are not bonded;
  - a tool configured to operably engage the billet outer material and billet inner material; and
  - an extrudate receiving channel configured to receive extrudate from the tool, the extrudate comprising extruded outer material and extruded inner material in at least one cross-section;

wherein:

  - the extruded outer material is the same material as the billet outer material, and the extruded inner material is the same material as the billet inner material; and the extruded inner material and the extruded outer material are bonded at an interface therebetween.
2. The assembly of claim 1 wherein the billet further comprises a billet intermediate material between the billet outer material and the billet inner material in the at least one cross-section.
3. The assembly of claim 2 wherein the extrudate further comprises extruded intermediate material between the extruded outer material and the extruded inner material in the at least one cross-section.
4. The assembly of claim 1 further comprising a mandrel extending from the billet containing assembly to the tool; wherein the mandrel extends through an opening in a die face of the tool.
5. The assembly of claim 1 further comprising a billet boundary material lateral of either the billet inner or outer material.
6. The assembly of claim 5 wherein:
  - the billet boundary material is lateral of the billet inner material, and
  - the billet boundary material is the same material as the billet outer material.
7. The assembly of claim 6 wherein the billet boundary material is lateral of the billet outer material.
8. The assembly of claim 5 wherein the billet boundary material comprises a different material than either or both of the billet inner or outer materials.
9. The assembly of claim 5 wherein in at least one cross-section the thickness of the inner and outer billet materials is different.
10. The assembly of claim 1, further comprising the billet.
11. A method for producing a multi-material shear assisted extrudate, the method comprising:
  - positioning a billet to be operably engaged with a tool, the billet comprising billet inner material and billet outer material, wherein the billet inner material and the billet outer material are not bonded; and
  - providing shear-assisted force to the tool operably engaged with the billet to form an extrudate comprising extruded inner material and extruded outer material, wherein:
    - the extruded outer material is the same material as the billet outer material, and the extruded inner material is the same material as the billet inner material; and the extruded outer material and the extruded inner material are bonded at an interface therebetween.
12. The method of claim 11 further comprising a billet intermediate material between the billet inner material and billet outer material.

9

**13.** The method of claim **12** wherein the billet intermediate material comprises a single material.

**14.** The method of claim **12** wherein the billet intermediate material comprises multiple different materials.

**15.** The method of claim **11** wherein the inner and outer billet material are about the same thickness in at least one cross-section.

**16.** The method of claim **15** wherein the extruded inner and outer materials are about the same thickness in at least one cross-section.

**17.** The method of claim **11** wherein the inner billet material is  $\frac{1}{10}$  to  $\frac{9}{10}$  the thickness of the outer billet material.

**18.** The method of claim **17** wherein the extruded inner material is  $\frac{1}{10}$  to  $\frac{9}{10}$  of the thickness of the extruded outer billet material.

**19.** The method of claim **11** wherein the extruded materials define bonded interfaces between different unbound billet materials.

**20.** A shear assisted extrusion assembly, the assembly comprising:

10

a billet containing assembly containing a billet, the billet comprising a billet outer material and a billet inner material in at least one cross-section, wherein the billet outer material and the billet inner material are not bonded;

a tool configured to operably engage the billet outer material and billet inner material;

a mandrel extending from the billet containing assembly to the tool, wherein the mandrel extends through an opening in a die face of the tool; and an extrudate receiving channel configured to receive extrudate from the tool, the extrudate comprising extruded outer material and extruded inner material in at least one cross-section;

wherein:

the extruded outer material is the same material as the billet outer material, and the extruded inner material is the same material as the billet inner material; and the extruded inner material and the extruded outer material are bonded at an interface therebetween.

\* \* \* \* \*